

## UNITED STATES PATENT OFFICE

2,280,721

## PROCESS OF DEVELOPING PHOTOGRAPHIC PICTURES

Andreas Schilling and Wilhelm Schneider, Dessau, and Gustav Wilmanns, Wolfen, Kreis Bitterfeld, Germany, assignors, by mesne assignments, to General Aniline & Film Corporation, New York, N. Y., a corporation of Delaware

No Drawing. Application November 14, 1939, Serial No. 304,321. In Germany November 24, 1938

3 Claims. (Cl. 95—88)

This invention relates to a process of developing photographic pictures and more particularly to the step of stopping the action of a photographic developer.

In ordinary black and white developing as well as in color-forming development the developer still acts on the photographic material when the same has been taken out of the developing bath and inserted into the subsequent washing bath. In the usual black and white development this feature is of no special consequence since only a certain increase in developed silver occurs, which may be recognized by a more intense blackening of the picture; the action of the developer subsequently to the development step proper is extremely undesirable in the process of color-forming development since it may easily cause a shifting of the color shades, that is a falsification of the color values, which is caused especially by the fact that the lower layers of a multi-layer photographic element are more intensely developed than the top layers. Besides this shifting of the color shades it is to be expected that under certain circumstances the ratio of gradation between the several layers is disturbed. In black and white development it has been usual to prevent this subsequent action of the developer by inserting in between the development and the fixing baths a stopping bath. These stopping baths were in general composed of dilute acids which neutralize the alkali of the developer and thereby interrupt the development of the silver halide.

In color-forming development the employment of such dilute acids as stopping baths is impossible since very dilute acids already act on the dyes formed by color-forming development. For instance the blue quinoneimine dyes are transformed into the red dyestuff salts by the acids and are partly completely destroyed. It has been found that the degree of acid which acts no longer on the dyes obtained by color-forming development is round about a pH-value higher than 3. This pH-value corresponds to very dilute acetic acid. If such very dilute acid solutions having a pH-value higher than 3 were employed for stopping the development it would be necessary to use so very dilute solutions that their stopping action would rapidly be neutralized by the alkali of the developer contained in the photographic layers. Furthermore, very weak acids do not yield water-resistant salts with the color-forming developer. Such stable salts, however, are necessary, since not only the action of the alkali must be stopped but the color-forming

developer must be dissolved from the layers in the form of a salt, it being known that the free base of dimethylamino-aniline, the usual color-forming developer, is rather difficultly soluble.

5 It is an object of the invention to overcome the above discussed difficulties.

A further object of the invention consists in the provision of an improvement in the color-forming development process.

10 A further object of the invention is to provide a novel photographic stopping bath.

Further objects of the invention will become apparent from the detailed specification following hereinafter.

15 We have found that the after-effects of the color-forming developer may be neutralized and the disadvantages of the stopping bath hitherto in use may at the same time be avoided, by employing as stopping baths solutions of primary or secondary salts polybasic organic acids the pH-value of which is not lower than 3 in solution. Advantageously a pH-value of between 3 and 5 is selected. It is known that the pH-value of such salt solutions which are known as buffer 20 solutions are independent of the concentration employed and it is therefore possible to employ solutions of high concentration or saturated solutions.

25 The stopping baths according to the present invention therefore act with very high efficiency and the effect of stopping the developer is produced rapidly and with certainty. Furthermore, the above described damaging of the dyes is avoided and the color-forming development compound is transformed into an easily 30 soluble form as a mixed salt and can easily be washed out of the layer.

35 The stopping baths may be employed in the color-forming development of layers containing dyestuff components as well as in color-forming development of photographic materials by means of developers containing the color-formers. Multi-layer materials with dyestuff components for color-forming development which have been 40 made fast to diffusion are preferred. Such dyestuff components are described in the following U. S. Patents 2,179,238, 2,178,612, 2,186,849 and 2,186,733, and in a number of other applications assigned to the present assignee.

## 50 Example

A multi-layer photographic element containing dyestuff components fast to diffusion is developed by color-forming development. At the end of the color-forming development it is immediately

immersed in a bath consisting of a solution of 10 per cent of primary sodium citrate. After being treated in the stopping bath for 1 minute the film is watered, bleached and fixed.

We claim:

1. In a process of producing color photographic pictures by color-forming development the step which comprises immersing the color photographic element immediately after the development thereof in a stopping bath containing a buffer solution of an acidic salt of a polybasic organic acid the pH-value of a solution of said salt being higher than 3.
2. In a process of producing color photographic pictures by color-forming development the step 15

which comprises immersing the color photographic element immediately after the development thereof in a stopping bath containing a buffer solution of an acidic salt of a polybasic organic acid the pH-value of a solution of said salt being from 3 to 5.

3. In a process of producing color photographic pictures by color-forming development the step which comprises immersing the color photographic element immediately after the development thereof in a solution containing about 10 per cent of primary sodium citrate.

ANDREAS SCHILLING,  
WILHELM SCHNEIDER,  
GUSTAV WILMANNS.